

Patented Jan. 10, 1928.

1,655,718 <sup>38</sup>

## UNITED STATES PATENT OFFICE.

HOWARD F. WEISS AND RALPH FORBUSH NORRIS, OF MADISON, WISCONSIN, AS  
SIGNORS, BY MESNE ASSIGNMENTS, TO C. F. BURGESS LABORATORIES, INC., OF  
DOVER, DELAWARE, A CORPORATION OF DELAWARE.

## WALL BOARD.

No Drawing.

Application filed June 17, 1924. Serial No. 720,510.

The present invention relates to wall boards suitable for use on the walls or ceilings of a room and having good heat insulating qualities. It is made from a mixture of 5 a filler and a binder which puffs into a porous rigid coherent mass under the action of heat and is provided with a facing of other material.

It is an object of the present invention to 10 produce a molded product composed for the most part of inorganic material, that product being light in weight, cheap in cost, and having a high porosity, and, consequently, a low thermal conductivity. The wall 15 boards of the present invention may be of the thickness and of the size of ordinary paper wall boards, and have a facing of paper on one or both sides. This sheet material can be put between the studding of a 20 building to serve in place of back plaster. It can also be used in sheets or blocks to form a wall or ceiling over which a layer of plaster or hard finish can be applied. Similarly it may be used as the exposed 25 surface of the wall, and before or after attachment to the studding may be decorated with enamel, paint, calcimine, or the like, applied directly to the mineral sheet, or applied to the paper facing or facings.

As set forth in a copending application, 30 Serial No. 720,511, filed June 17, 1924, when an intumescent binder such as a soluble alkali silicate, hide glue or cornstarch is mixed with a filler and subjected to the action of heat, the mass expands or puffs up 35 and ultimately hardens into a firm strong body filled with air cells or pores, the size and distribution of which we find can to a large extent be controlled. Unless the expansion or puffing of the material is 40 restricted as in a closed mold or form, the expansion is likely to proceed so far that the resultant product will be too light and frothy to accomplish the ends now desired 45 by us.

The density and the physical characteristics of wall boards made from such material by the application of heat in a mold will depend in part on the relative percentages of 50 binder and filler; in part on the size of the mold with respect to the amount of raw

material put in for heat treatment, and in part on the chemical and physical characteristics of the filler. By suitable control of these factors, and of the temperature and 55 duration of heat treatment, a wide range may be obtained in the physical characteristics of the product.

Various fillers can be used, such, for example, as crushed dolomite, limestone, blast 60 furnace or other slag, kaolin, slate, asbestos, either fibrous or powdered various clays, slag wool, powdered silica, ochre, tripoli, volcanic ash, pumice, kieselguhr, ashes, or various mixtures thereof. <sup>65</sup>

Instead of using a filler that is entirely of mineral origin, there may be incorporated in the mixture, before heat treatment thereof, organic materials, such as wood flour, wood pulp, cork, sawdust, charcoal, wood 70 slivers, or shredded bark. Such organic materials may be used to alter the properties to the degree desired. For certain purposes the filler may be entirely of organic origin. <sup>75</sup>

By way of illustration we give below detailed instructions for proceeding in accordance with the method of the present invention.

An alkali silicate, such as sodium silicate, 80 having a density of about 42.5° Bé. is intimately mixed as in a mixer with a filler to form a dough having a consistency about like that of putty. The amount of filler varies with its character, for example in using dolomite the filler constitutes about 60% of the weight of the wet mix, while in using kieselguhr or sifted coal ashes, the filler constitutes only 20% of the weight of the wet mix. When the board or panel is to have 90 a paper facing on both sides, the dough or mix thus formed is spread upon a sheet of paper either in an even layer or as strips. (an even layer having a depth of  $\frac{1}{16}$  to  $\frac{1}{8}$ " will form a board approximately  $\frac{5}{16}$ " in 95 thickness). A second sheet of paper is placed on top of the dough so that the product in its green condition consists of two sheets or strips of paper with a layer of dough between. The paper we have been using is an ordinary chip board rather heavily 100 sized so that it will be water resistant and

tough, although, of course, other kinds of paper can be used. The green sheet is then slid between two steam heated iron platens spaced a distance equal to the thickness desired for the finished board, say, for instance,  $\frac{15}{16}$ ". The steam platens can be heated with steam at a pressure of about 25 to 100 lbs., but a temperature of more than about  $170^{\circ}$  C. should not be employed to avoid charring of the paper facing. The application of heat of about that temperature causes the dough to puff up and force the upper sheet of paper against the upper platen. During this heating process steam is driven off from the mixture, particularly along the edges of the board. Some dough also may escape around the edges of the board without disadvantage. During this heating and expanding process, and the driving off of water from the mixture the silicate undergoes a radical physical change, and there may even be a chemical reaction between the silicate and the filler. In about thirty (30) minutes the dough has puffed sufficiently and sufficient moisture has been driven off so that the board in its puffed and porous condition is stiffer than when it was wet or green, although it still is somewhat plastic. The hot board is then slipped from between the platens and pressed between two rigid surfaces and there allowed to cool so that when it has cooled it is held sufficiently flat. It is then in a stiff hardened and porous condition, and can be trimmed with saws and cut to the desired dimensions.

If the board is to be faced with paper on one side only, a greased iron sheet is substituted for one of the paper sheets.

The tenacity with which the composition sticks to the paper sheets is one of the important characteristics of the paper faced board, for there is no tendency for the sheets to blister or strip away from the mineral filler. The paper is very tenaciously held, thereby strengthening the board and adding to its resistance against chipping during shipment, or while nails are being driven through it into the studding. In cross section the inorganic core of the finished board is not unlike in appearance the cross section of a loaf of fine grained bread.

We have found that a soap, such as sodium resinate, stearate and the like, or material such as oleic acid which will be saponified by the silicate, can be advantageously added to the batch, for controlling the size and distribution of the air bubbles or cavities. For instance, with a mixture of sodium silicate and ashes in about equal parts by weight there may be added soap to the extent of less than one-half of one percent by weight. This soap addition makes the bubbles smaller, but more numerous, and reduces the apparent density of the finished product. Presumably these holes or cav-

ties represent spaces where steam was trapped in the mix during the puffing procedure.

Using 2.7 parts by weight of sodium silicate of  $42.5^{\circ}$  Bé., 4.0 parts of finely ground dolomite, then mixing to a stiff dough, there may be produced, after heat treatment, a strong product weighing 45.0 lbs. per cu. ft. By increasing the proportion of dolomite a heavier product will result. Thus by adding 6.0 parts of dolomite in the mix indicated, a product weighing  $62\frac{1}{2}$  lbs. per cu. ft. may be made. It is not advantageous to make a denser product.

We have found the following batch to give excellent results, the percentage given being parts my weight:—

39%  $42.5^{\circ}$  Bé. sodium silicate solution.

58% powdered dolomite.

29% fine sawdust.

0.1% sodium oleate.

Dolomite, which consists essentially of calcium and magnesium carbonates in varying proportions up to about 55% and 45% respectively, is widely distributed throughout the United States, and is available in large quantities and low cost in the State of Illinois and in neighboring States. (See Bulletin 46 of the State of Geological Survey of Illinois entitled "Lime stone resources of Illinois".)

The wall board made as above described can be sawed and handled much as plaster or gypsum board is handled, and has the advantage thereover that it is lighter in weight and far more porous. Not only is the material of low conductivity for heat and sound, but it has a low water absorption coefficient and if necessary can be waterproofed.

We claim:—

1. A wall-board characterized by the tenacity between the core and the facing comprising a mixture of an intumescent binder and a filler, puffed by heat to a highly porous coherent body, and having a facing held in place by the intumesced binder.

2. A wall-board characterized by the tenacity between the core and the facing comprising a mixture of an alkali silicate and a filler, puffed by heat to a highly porous body, and having a facing held in place by the intumesced binder.

3. A wall-board characterized by the tenacity between the core and the facing weighing not more than  $62\frac{1}{2}$  pounds per cu. ft. comprising a mixture of an alkali silicate and a filler, puffed by heat, and having a facing held in place by the intumesced binder.

4. A wall-board characterized by the tenacity between the core and the facing comprising a mixture of an alkali silicate and a filler, puffed by heat to a highly porous body of a fibrous character, and having a facing held in place by the intumesced binder.

5. A wall-board characterized by the tenacity between the core and the facing comprising a mixture of an alkali silicate and a heavy mineral filler, and a porous filler, puffed by heat to a highly porous product, and having a facing held in place by the intumesced binder.
6. A wall-board characterized by the tenacity between the core and the facing comprising a mixture of sodium silicate and crushed dolomite puffed by heat to a highly porous product and having a paper facing held in place by the intumesced binder.
7. A wall-board characterized by the tenacity between the core and the facing comprising a mixture of an alkali silicate, a filler, and a soap, puffed by heat to a rigid mass, and having an adherent facing.
8. A wall-board characterized by the tenacity between the core and the facing comprising a mixture of alkali silicate, a mineral filler, and sodium oleate, puffed and hardened by heat, and having an adherent facing.
9. A wall-board characterized by the tenacity between the core and the facing comprising a mixture of an alkali silicate and about 60% of a crushed dolomite based on the wet weight of the mixture, puffed by heat to a rigid mass, and having an adherent facing.
10. A wall-board characterized by the tenacity between the core and the facing comprising a mixture in parts by weight of 39% 35 42.5 Bé. sodium silicate solution, 58% powdered dolomite, 2.9% fine sawdust, 0.1% sodium oleate puffed by heat to a porous body, and having an adherent facing of paper.
11. The process of making wall-board having a high degree of tenacity between the core and the facing which comprises mixing an intumescent binder with a filler, subjecting the batch so formed to heat while confined between paper liners until the material puffs to a porous coherent product and adheres to the paper.
12. The process of making wall-board having a high degree of tenacity between the core and the facing which comprises mixing sodium silicate with a filler, introducing the batch so formed between paper liners and then heating by contact with hot plates until the material puffs to a porous coherent product and adheres to the paper.
13. The process of making wall-board having a high degree of tenacity between the core and the facing which comprises mixing sodium silicate with crushed dolomite, introducing the batch so formed in a relatively thin layer between paper liners, and then confining the material and subjecting to heat until the material puffs to a porous coherent product and adheres to the paper.
14. The process of making wall-board having a high degree of tenacity between the core and the facing which comprises mixing an intumescent binder with a filler, introducing the batch so formed into a mold having a paper lining and there heating it until the material puffs to a porous coherent product, and adheres to the paper.
15. The process of making wall-board having a high degree of tenacity between the core and the facing which comprises mixing an alkali silicate with a filler, introducing the batch so formed into a mold having a paper lining and there heating it until the material puffs to a porous coherent product, and adheres to the paper.
16. The process of making wall-board having a high degree of tenacity between the core and the facing which consists in mixing an alkali silicate with a filler, introducing the batch so formed into a mold lined with paper, and there heating until the material puffs to a weight less than 62½ lbs. per cu. ft. and adheres to the paper.
17. The process of making wall-board having a high degree of tenacity between the core and the facing which consists in mixing alkali silicate with a mineral filler, introducing the batch so formed into a mold lined with paper, and then heating at about 150° C. until the material puffs and hardens to a rigid porous mass and adheres to the paper.
18. The process of making wall-board having a high degree of tenacity between the core and the facing which consists in mixing an alkali silicate with a filler to form a batch of dough-like consistency, introducing the batch into a mold lined with paper and heating at about 150° C. for about 30 minutes to puff and harden the batch; and cause it to adhere to the paper.
19. The process of making wall-board having a high degree of tenacity between the core and the facing which consists in mixing an alkali silicate with a mineral filler to form a batch of dough-like consistency, introducing the batch into a mold lined with paper and heating at about 150° C. for about 30 minutes to puff and harden the batch; and cause it to adhere to the paper.
20. The process of making wall-board having a high degree of tenacity between the core and the facing which consists in intimately mixing an alkali silicate with a filler and a soap, introducing the batch so formed into a mold lined with paper and heating to puff and harden the batch, and cause it to adhere to the paper.
21. The process which consists in intimately mixing about 2.7 parts alkali silicate with about 4.0 parts crushed dolomite by weight, mixing the batch to a doughy consistency, introducing it into a metal mold and there heating at about 150° C. for about 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970

thirty minutes to puff and harden said dough, and cause it to adhere to the paper.

22. The process of making wall-board having a high degree of tenacity between the core and the facing which comprises mixing an alkali silicate with a filler, introducing the batch so formed into a mold lined on one face with paper, the other face

being of greased metal, and heating to puff and harden the batch and cause it to adhere to the paper.

In testimony whereof we affix our signatures.

HOWARD F. WEISS.  
RALPH FORBUSH NORRIS.